

## UNITED STATES PATENT OFFICE

1,960,551

CELLULOSIC PRODUCTS AND METHOD OF  
MAKINGGeorge A. Richter, Berlin, N. H., assignor to  
Brown Company, Berlin, N. H., a corporation  
of MaineNo Drawing. Application March 24, 1931,  
Serial No. 525,037

18 Claims. (Cl. 260—10)

This invention relates to the manufacture of cellulosic products wherein cellulose fiber of the type of cotton or chemical wood pulp serves as the starting material. Among the cellulosic products comprehended by the present invention are papers and cellulose esters or derivatives, such as the xanthate, nitrate, and acetate.

In making papers and cellulose derivatives, it is desirable to use as a raw material white cellulose fiber of high purity and stability, such as cotton or bleached chemical wood pulps of high alpha cellulose content. In some instances, too, a pulverulent cellulose derived from such fiber may be put to use to great advantage. Thus, when mechanically pulverized cellulose fiber of the kind described is incorporated into papermaking furnishes, the opacity and surface characteristics of the finished paper may be easily and economically controlled by the use of a suitable amount of cellulose powder of the appropriate particle size. The cellulose powder constitutes an excellent filler for high grade papers and may so be applied as to appear throughout the body of the paper or as a surface coating. For instance, as already indicated, the powder may be incorporated into papermaking furnishes, including a high grade rag stock, the usual chemical wood pulps such as sulphite, or refined white wood pulps of high alpha cellulose content, together with, if desired, the usual papermaking ingredients, such as rosin size and mineral fillers. On the other hand, the cellulose powder, together with suitable adhesives such as dextrine paste, glue, rosin size, or the like, may be spread as a coating on either or both faces of the fabricated paper. Depending on the fineness of the cellulose powder, the surface qualities of the paper may be varied from a comparatively rough finish, known as "egg shell" to a perfectly smooth or flat finish, such as is sometimes desired in printing or writing papers. Cellulosic powder or waterleaf papers containing such powder are eminently suitable for conversion into cellulose derivatives such as the xanthate, particularly as cellulose in finely divided condition is highly reactive with con-

the market. The bulk or sheeted pulp is initially transformed into a non-hydratable condition, by which I mean that the cellulose is so altered that it does not take on a slimy or gelatinous condition when beaten in water. This can well be accomplished by mercerizing the fibers as with a caustic soda solution. The solution employed may be of a concentration designed to mercerize the pulp at the particular temperature at which it is used. Should the treatment be carried out at room temperature (about 30° C.), as is usually preferable, the solution should be of about 18% caustic soda content. When lower treating temperatures are resorted to, the solution may be of a strength below 18%, since lower temperatures are conducive to mercerization with weaker solutions. When bulk pulp is used, the mercerizing solution may be uniformly mixed with the pulp to form a stock suspension of about 10%. After the required period of exposure to the action of the mercerizing solution, the excess liquor serving as a suspension vehicle may be removed as by a thickener or in a centrifuge, whereupon the thickened, mercerized stock may be washed free from residual alkali, as in a countercurrent pulp washer. When drier sheets are being handled, they may be subjected to processing steps similar to those constituting the initial steps of the usual viscose-rayon process; that is, the sheets may be steeped in a mercerizing solution for an appropriate period of time, and the excess solution imbibed by the sheets then pressed therefrom. Rather than maintaining a fixed amount of alkali in the pressed, mercerized sheets, as in the viscose-rayon process, however, the alkali content of the sheets is, in accordance with the present invention, removed by washing. The mercerizing solution, in addition to transforming the fiber into a non-hydratable condition, effects a purification thereof, as non-alpha cellulose components of the fiber are soluble and go into solution in the mercerizing liquor. This purification may be quite marked when an ordinary commercial wood pulp, such as bleached sulphite, serves as the raw material. The purification effected by the mercerizing liquor is enhanced by the subsequent washing operation, particularly when hot wash water is relied upon to remove residual alkali, as the hot alkaline solution formed during washing is an excellent solvent for various non-alpha cellulose components associated with the fiber. The washed, mercerized pulp, either in bulk or sheet form, may then be dumped into a beater engine with the necessary quantity of circulating water, and the aqueous stock sus-

In accordance with the present invention, I may start with cotton, chemical wood pulp, or other preferably white cellulose fiber of high purity and stability, as raw material. The pulp may be in bulk condition or in thick sheets known commercially as "drier sheets". This latter form is that which chemical wood pulps, especially high grade refined wood pulps of high alpha cellulose content, are likely to assume when put on

pension thus formed subjected to hard beating until the fibers have been reduced to a pulverulent state. The beater roll cuts and bruises the mercerized fibers with little, if any, hydrating or gelatinizing action thereupon, so that the stock is gradually transformed into an aqueous slurry lacking the marked slimy or gelatinous feel of ordinary, well-beaten papermaking stock. The aqueous slurry may be incorporated into paper-  
5 stocks while they are undergoing beater action, and the mixture formed into papers of a sized or waterleaf character. It may also be used together with suitable water-soluble adhesives for coating papers, fabrics, or the like. If desired, 10 however, the powdered cellulose in the aqueous slurry may be separated from its excess aqueous component, as by settling or filtration, and the separated powder then dried for storage or shipment. After separation from the aqueous ve-  
15 hicle in which it is suspended, the concentrated or still wet powder may be pressed into coherent cakes or masses, and finally dried in such form for packaging. The dry product constitutes a step product for storing or marketing, and as such 20 may be supplied to papermaking and cellulose de-  
25 rivative manufacturers.

The principles of the present invention extend to other forms of non-hydratable cellulose, for instance to celluloses regenerated as from viscose syrup. In this connection, artificial silk waste, such as viscose-rayon yarns which have been spoiled or damaged in processing, may serve as the source of the powdered cellulose of the present invention. A feature of importance re-  
30 siding in the present invention is that mercerized cellulose fiber or other non-hydratable cellulose may be pulverized in the presence of an aqueous medium by standard papermaking machines, such as beater engines. It is, however, within the 35 contemplation of my invention to practise a dry, rather than a wet, pulverizing operation, as in ball mills, to which mills the mercerized or other non-hydratable cellulose may be supplied in bulk form or as sheets. Pulverization may also be ac-  
40 complished in the presence of non-aqueous wetting media, such as benzol, which may be readily volatilized from the cellulose powder after the major portion of such media has been removed, as by filtration, from the slurry of cellulose pow-  
45 der. The cellulose powder may be of a particle size ranging from about 40 to 200 mesh, or even finer. In some instances, the powder may be composed of particles of varying sizes, as when a batch reduced to particles passing through a 50 40-mesh sieve is blended with a batch of fibers reduced to particles passing through a 200-mesh sieve. In some instances, raw or unbleached wood pulps may serve as the starting material, in which case such pulp undergoes a marked 55 refinement, as well as mercerization, by contacting with the alkaline mercerizing liquor. The mercerizing liquor may contain sufficient oxidants, such as hypochlorite, to bleach or whiten the pulp; or the mercerized, washed pulp may 60 receive an independent bleaching treatment with suitable bleach liquors before the pulverizing operation. In any event, the pulverized product is preferably a pure white one of high stability and composed substantially only of alpha cellulose.  
65 70 In carrying out the mercerization of the fiber prior to its pulverization in accordance with the present invention, it is possible to add chemicals, such as oxidizing or reducing agents, to the mercerizing liquor, to effect reaction on impurities or coloring matters associated with the fiber.  
75

For instance, oxidants, such as hypochlorites or permanganates, may be added to the mercerizing liquor to enhance the whiteness and brightness of color in the mercerized fiber, as well as to render the fibers more easily disintegratable into a powder under pounding action, as in a ball mill. So, too, reducing agents, such as sodium sulphide, may constitute additions to the mercerizing liquor, particularly when the liquor em-  
80 ployed is one derived from the smelted sodium compounds produced during the recovery operations practised in a kraft mill, which operations lead to the production of a liquor containing sodium sulphide, as well as caustic soda. In some instances, the mercerized fiber may be one which is aged in accordance with the practice fol-  
85 lowed in making viscose syrup such as intended for rayon manufacture; that is, the pulp in sheet form may be submerged in a mercerizing liquor, then pressed free of excess liquor, then fluffed, and permitted to age in fluffed condition under controlled temperature conditions. Inasmuch as the aged pulp contains alkali and has been some-  
90 what degraded during ageing, it is then washed free of alkali and is preferably digested in a re-  
fining solution of hot, dilute alkali, as disclosed and claimed in my application Ser. No. 132,319, filed August 28, 1926. The washed, aged, and preferably refined cellulose fiber may then be dried and in such condition serve as the raw material for the preparation of the powdered cellulose of the present invention.  
95

So far as certain subject matter is concerned, this is a continuation in part of my application Serial No. 196,135, filed June 2, 1927, which has 100 matured into Patent No. 1,842,689, dated Jan. 26, 1932.

What I claim is:

1. A paper containing powdered, non-hydratable cellulose fiber whose particle size is not greater than about 40 mesh.  
115
2. A paper containing powdered, mercerized cellulose fiber whose particle size is not greater than about 40 mesh.  
120
3. A process which comprises converting cel-  
lulose fiber into a non-hydratable condition and  
then pulverizing the fiber in the presence of  
water to a particle size not greater than about 40  
mesh.  
125
4. A process which comprises mercerizing cel-  
lulose fiber and then pulverizing the mercerized  
fiber in the presence of water to a particle size  
not greater than about 40 mesh.  
130
5. A process which comprises incorporating  
pre-powdered, non-hydratable cellulose fiber into  
an aqueous suspension of papermaking stock, and  
then forming paper from the mixture.  
135
6. A process which comprises incorporating  
pre-powdered, non-hydratable cellulose fiber into  
an aqueous suspension of papermaking stock, forming  
paper from the mixture, and converting  
the paper into cellulose esters.  
140
7. A process which comprises pulverized non-  
hydratable cellulose fiber in the presence of wa-  
ter to a particle size not greater than about 40  
mesh, and converting the powder into cellulose  
esters.  
145
8. A process which comprises pulverizing mer-  
cerized cellulose fiber in the presence of water  
to a particle size not greater than about 40 mesh,  
and converting the powder into cellulose esters.  
150
9. A process which comprises pulverizing mer-  
cerized cellulose fiber, incorporating the powder  
into an aqueous suspension of papermaking stock,  
150

- forming paper from the mixture, and converting the paper into cellulose esters.
10. A process which comprises steeping cellulose fiber in a mercerizing liquor, removing excess liquor from the fiber, washing the fiber, and beating the mercerized and washed fiber in water to form an aqueous slurry of powdered cellulose of a particle size not greater than about 40 mesh.
- 10 11. A process which comprises pulverizing mercerized cellulose fiber in water to form an aqueous slurry, incorporating the slurry into an aqueous suspension of papermaking stock, and forming the mixture into paper.
- 15 12. A process which comprises pulverizing mercerized cellulose fiber in water to form an aqueous slurry, removing excess water from the slurry to concentrate the pulverized cellulose, and drying the concentrate.
- 20 13. A process which comprises pulverizing mercerized cellulose fiber in water to form an aqueous slurry, removing excess water from the slurry to concentrate the pulverized cellulose, pressing the concentrate into cake form, and 25 drying the cake.
14. A process which comprises converting cellulose fiber into a non-hydratable condition and then pulverizing the fiber to a particle size not greater than about 40 mesh.
15. A process which comprises mercerizing cellulose fiber and then pulverizing the mercerized fiber to a particle size not greater than about 40 mesh. 80
16. A cellulose product consisting substantially entirely of powdered non-hydratable cellulose fiber of the character of cotton and chemical wood pulp, said powder being of a particle size not exceeding about 40 mesh. 85
17. A cellulose product consisting substantially entirely of powdered, mercerized cellulose fiber of the character of cotton and chemical wood pulp, said powder being of a particle size not exceeding about 40 mesh. 90
18. A cellulose product consisting substantially entirely of powdered, regenerated cellulose, said powder being of a particle size not exceeding about 40 mesh. 95

GEORGE A. RICHTER.

100

- 30
- 35
- 40
- 45
- 50
- 55
- 60
- 65
- 70
- 75
- 80
- 85
- 90
- 95
- 100
- 105
- 110
- 115
- 120
- 125
- 130
- 135
- 140